

# UNITED STATES PATENT OFFICE.

MAX BECKE AND ALBERT BEIL, OF HÖCHST-ON-THE-MAIN, GERMANY, AS-SIGNORS TO THE FARBWERKE, VORMALS MEISTER, LUCIUS & BRÜNING, OF SAME PLACE.

## PROCESS OF DYEING UNIONS.

SPECIFICATION forming part of Letters Patent No. 623,697, dated April 25, 1899.

Application filed August 5, 1897. Serial No. 647,220. (Specimens.)

*To all whom it may concern:*

Be it known that we, MAX BECKE, chemist, a citizen of the Empire of Austria-Hungary, and ALBERT BEIL, chemist, a citizen of the Empire of Germany, residing at Höchst-on-the-Main, in the Empire of Germany, have invented a new and useful Improvement in Dyeing Half-Wool with Basic Azo Dyestuffs in an Acid-Bath, (for which Letters Patent were granted to us in France, No. 264,579, dated March 2, 1897, and in England, No. 5,119, dated February 25, 1897,) of which the following is a specification.

The simultaneous working of wool and cotton is of great importance in the manufacture of spun and woven goods of all kinds. Dyers accordingly have endeavored to find suitable methods for the equal dyeing of those two fibers—that is to say, to improve the present system. These efforts, however, have not been thoroughly successful, the present methods being very deficient.

Two methods are now mostly employed in dyeing half-wool. The one consists in first dyeing the wool with acid dyestuffs in an acid-bath; secondly, in mordanting the cotton in cold baths containing tannin; thirdly, in fixing the absorbed tannin by passing the material through fixing-baths, (mostly antimonal or ferruginous,) and, finally, in dyeing the cotton thus previously mordanted with basic dyestuffs in a fourth bath to the desired shade. This method is cumbersome and uncertain on account of its many operations and the difficulty of producing in two dye fluids the shade desired on wool and cotton.

When the coal-tar industry put on the market the tetrazo dyestuffs derived from para-diamins, the second important method for dyeing half-wool was found and applied. The said diamine dyestuffs possess, as is known, the property of dyeing wool as well as cotton in neutral or weak alkaline baths.

By a proper choice of dyestuffs, an appropriate regulation of the temperature when dyeing, and the addition of quantities of more or less alkaline salts it is possible to produce

the most varied shades on half-wool in a single bath. This method is popular on account of its simplicity; but it has one great drawback—namely, that the quality of the goods suffers enormously, as the fiber of the wool boiled in neutral or mostly alkaline baths loses its most valuable properties. This disadvantage is so great that in the case of many articles, and after vain efforts with this single-bath method, half-wool dyers have returned to the old and more troublesome system.

We have succeeded in finding a method for dyeing half-wool combining the advantages of the single-bath method with the complete preservation of the properties of the valuable wool material, thus proving to be an essential technical progress in the half-wool industry. We have found that such strongly-basic disazo dyestuffs resulting from the linking of at least three aromatic residues and containing as a component an aromatic ammonium base or amidobenzylamin or their derivatives, as also basic safranin azo dyestuffs, are easily fixed on half-wool in an acid-bath, preferably in a sulfuric-acid bath, dyeing cotton and wool equally. The simple azo dyestuffs produced from an aromatic ammonium base or amidobenzylamin or their derivatives do not possess this property, which is first obtained by the joining of a second residue combined with an azo group, yet the strongly-basic character of the dyestuff must be retained, as the presence of acid groups reduces the affinity of the fiber and sulfo groups, mostly neutralizing the same.

The following dyestuffs have been found suitable for the above purpose: first, the disazo dyestuffs having as first component an ammonium base (trialkyl - meta and para- amidophenylammonium, para-methyl-ortho- amidophenyl-trialkylammonium, trialkyl-ortho- and para - amidobenzylammonium or dialkyl-ortho- and para-amidobenzylamin) and as component in middle position alpha-naphthylamin, para - xylidin, symmetrical meta-xylidin, meta - toluidin, meta - chloranilin, ortho-chloro-meta-toluidin, ortho-anisidin,

ortho-amido-para-cresolmethylether, alpha-amido-beta-naphthoether, and as component in final position dimethyl and diethyl-metamido-phenol, phenylene- and toluylene-diamin, chrysoidin, resorcinol, beta-naphthol phenyl and tolyl-beta-naphthylamin amidonaphthols, pyrazolones, besides, second, those secondary basic disazo dyestuffs which are obtained by the action of one molecule each of two different diazo compounds (of which one must be the diazo compound of an ammonium base or of a dialkylbenzylamin, while the other, for instance, may be acetyl-para-phenylenediamin, meta- and para-nitranilin, alphanaphthylamin, anilin, &c.) to one molecule of double combining phenols, amido phenols, or diamin—such as resorcinol, dialkyl-metamidophenol, meta-phenylenediamin; third, these disazo dyestuffs obtained by the action of the diazo compound of an amidoazo body upon 2.7 oxynaphthalin trialkylammonium; fourth, the basic safraninazo dyestuffs obtained by the action of diazo-safranins or diazo-alkylsafranins upon phenols, amidophenols, naphthols, dioxynaphthalenes, amidonaphthols, amidonaphthol ethers, amines, or diamines.

For the dyeing of half-wool the bath is filled with two per cent. of sulfuric acid relatively to the weight of the goods, with the carefully-prepared solution of the above-mentioned dyestuff in the quantity suitable to the required shade, as well as with five to twenty per cent. of Glauber's salt. The previously cleaned and wetted material is introduced into the bath at 40° to 50° centigrade, which is then brought to boiling while being correspondingly worked, the boiling to continue for one hour. The material is slightly washed, in case of dark colors, with argillaceous or fullers' earth and dressed in the usual manner.

Instead of sulfuric acid sodium bisulfate may be employed. If the wool is intended to be much lighter than the cotton, then the sulfuric acid is partly or wholly substituted by oxalic acid.

The attraction for wool is increased by additions of neutral salts, such as Glauber's and common salt.

Other acids, as hydrochloric or acetic acid, as well as acid salts, alum, or tartar, may be used, giving similar yet not quite so good results as sulfuric acid. The after-shading of wool and cotton may be done in the boiling bath with the said basic azo dyestuffs and such other dyestuffs as do not give with the former any insoluble precipitates.

This method permits a short, easy, and sure working, as well as the exact point of the intended shades. The boiling in an acid-bath preserves the natural feel, gloss, and solidity of the wool and improves thereby the half-wool material to be dyed.

The process may be illustrated by the following examples:

I. *Fashion color upon twenty kilos, equaling three pieces, of Orleans, each of one hundred meters.*—The bath is prepared with:

|                                      |                                                                                          |    |
|--------------------------------------|------------------------------------------------------------------------------------------|----|
| 60 grams half-wool red M. T.         | Disazo dyestuffs from trimethyl-metamido-phenylammonium + meta-toluidin + beta-naphthol. | 70 |
| 100 grams half-wool yellow A         | Dyestuff from trimethyl-metamido-phenylammonium and meta-nitrobenzene azoresorcinol.     |    |
| 40 grams half-wool green B           | Dyestuff from diazo-diethyl-safranin and dimethylanilin.                                 | 75 |
| 400 grams sulfuric acid at 66° Baumé |                                                                                          |    |

The previously dressed and wetted material is introduced at 50° centigrade, brought to boil within one-half hour, and kept at this temperature for a further one-half hour. Then the steam is stopped and the dyeing is continued till all the cotton, as is required with these goods, takes a darker hue than the wool. Thereupon the pieces are taken out, washed, slung, slightly dressed with gelatin, dried, and pressed.

II. *Gray upon nine kilos, equaling one piece forty-five meters, half-wool zanella.*—The bath is prepared with:

|                              |                                                                                       |    |
|------------------------------|---------------------------------------------------------------------------------------|----|
| 45 grams half-wool yellow A  | Disestuff from trimethyl-metamido-phenylammonium and meta-nitrobenzene azoresorcinol. | 90 |
| 27 grams half-wool red M. T. | Dyestuff from trimethyl-metamido-phenylammonium + meta-toluidin + beta-naphthol.      |    |
| 50 grams half-wool green B   | Dyestuff from diazo-diethyl-safranin and dimethylanilin.                              | 95 |
| 9 grams half-wool blue R     | Dyestuff from diazo-safranin-beta-naphthol.                                           |    |
| 900 grams Glauber's salt     |                                                                                       |    |
| 180 grams sulfuric acid      |                                                                                       |    |

The previously-dressed material is introduced at 50° centigrade, brought to boil within one-half hour, and kept at this temperature till the cotton is sufficiently dyed, completing the dyeing process by another half-hour's boil.

III. *Brown upon nine kilos, equaling one piece forty-five meters, half-wool zanella.*—The bath is prepared with:

|                              |                                                                                      |     |
|------------------------------|--------------------------------------------------------------------------------------|-----|
| 215 grams half-wool brown A  | Dyestuff from trimethyl-metamido-phenylammonium alpha-naphthylamin and chrysoidin.   | 110 |
| 67 grams half-wool green B   | Dyestuff from diazodiethyl-safranin and dimethylanilin.                              |     |
| 20 grams half-wool red M. T. | Dyestuff from trimethyl-metamido-phenylammonium + meta-toluidin and beta-naphthol.   |     |
| 13 grams half-wool yellow A  | Dyestuff from trimethyl-metamido-phenylammonium and meta-nitrobenzene azoresorcinol. | 115 |
| 9 grams half-wool blue R     | Dyestuff from diazo-safranin + beta-naphthol.                                        |     |
| 900 grams Glauber's salt     |                                                                                      |     |
| 180 grams sulfuric acid      |                                                                                      |     |

The previously-dressed material is introduced at 50° centigrade, brought to 85° centigrade within one-half hour, and kept at this temperature till the cotton is sufficiently dyed, completing this dyeing process by a further one-half hour's boil.

IV. *Copper color upon fifty kilos Vigogne*

yarn, (fifty per cent. wool, fifty per cent. cotton.)—The bath is prepared with:

5 1.250 kilos half-wool brown R. { Azo dyestuff from trimethylmeta-aminophenyl ammonium, meta-toluidin, and chrysoidin.  
5     kilos Glauber's salt  
1     kilo sulfuric acid of 66° Baumé.

The previously well-washed yarn is introduced at 50° centigrade, brought to boil within one-half hour, and dyed for three-quarters of an hour while being well worked.

Having thus described our invention, we claim as new and desire to protect by Letters Patent—

15 A process of dyeing half-wool, which consists in subjecting the wool and cotton in half-woolen goods simultaneously in one acidulated bath to the action of basic polyazo dyestuffs and safraninazo dyestuffs, substantially as set forth.

20 In testimony that we claim the foregoing as our invention we have signed our names in presence of two subscribing witnesses.

MAX BECKE.  
ALBERT BEIL.

Witnesses:

HEINRICH HAHN,  
ALFRED BRISBOIS.